# EUROPEAN PATENT APPLICATION

(11) **EP 4 696 813 A1**
(43) Date of publication of application: **18.02.2026**
(21) Application number: 24788844.9
(22) Date of filing: 12.04.2024
(51) Int. Cl.: C23C 22/00, C21D 8/12, C21D 9/46, C22C 38/00, C22C 38/60

(54) **GRAIN-ORIENTED ELECTRICAL STEEL SHEET AND METHOD FOR FORMING INSULATING COATING FILM**

(30) Priority: 12.04.2023 JP 2023064836
(71) Applicant: NIPPON STEEL CORPORATION, Chiyoda-ku Tokyo 100-8071 (JP)
(72) Inventor: TAKEDA, Kazutoshi, Tokyo 100-8071 (JP); TAKATANI, Shinsuke, Tokyo 100-8071 (JP); KATAOKA, Takashi, Tokyo 100-8071 (JP); KOGAKURA, Yuuki, Tokyo 100-8071 (JP)
(74) Representative: Vossius & Partner Patentanwälte Rechtsanwälte mbB
(86) International application number: PCT/JP2024/014848
(87) International publication number: WO 2024/214822

(57) **Abstract**

This grain-oriented electrical steel sheet includes a base steel sheet and an insulating coating formed on a surface of the base steel sheet, the insulating coating is formed on a side of the base steel sheet, and includes an intermediate layer containing a crystalline metal phosphate and one or more of amorphous silica, an inorganic filler, and a metal oxide, and a tension coating layer formed on a surface side of the insulating coating, and an average particle diameter of one or more of the amorphous silica, the inorganic filler, and the metal oxide is 10 to 500 nm.

## Description

### TECHNICAL FIELD

The present invention relates to a grain-oriented electrical steel sheet and a method for forming an insulating coating.

Priority is claimed on Japanese Patent Application No. 2023-064836, filed April 12, 2023, the content of which is incorporated herein by reference.

### BACKGROUND ART

A grain-oriented electrical steel sheet is mainly used for a transformer. The transformer is continuously magnetized for a long period of time from installation to disposal and continues to generate energy loss. Therefore, energy loss when the transformer is magnetized by alternating current, that is, iron loss is a main index for determining performance of the transformer.

In order to reduce iron loss of the grain-oriented electrical steel sheet, many techniques have been developed so far from a viewpoint of (a) increasing development in the { 110}<001> orientation (Goss orientation), (b) increasing the content of a solid solution element such as Si to increase electric resistance of the steel sheet, or (c) reducing the sheet thickness of the electrical steel sheet.

In addition, applying tension to the steel sheet is effective for reducing iron loss. It is an effective means for reducing iron loss to form a coating made of a material having a thermal expansion coefficient smaller than that of the steel sheet on a sheet surface at a high temperature. A forsterite film (inorganic coating) having exceptional coating adhesion, generated by a reaction between an oxide on a sheet surface and an annealing separator in a finishing annealing step of an electrical steel sheet is a coating capable of applying tension to the steel sheet.

For example, a method for forming an insulating coating by baking a coating liquid mainly containing colloidal silica and a phosphate on a sheet surface, disclosed in Patent Document 1, is an effective method for reducing iron loss because the method has a large effect of applying tension to the steel sheet. Therefore, a general method for manufacturing a grain-oriented electrical steel sheet is to leave the forsterite film generated in the finishing annealing step and to form an insulating coating mainly containing a phosphate on the forsterite film.

However, in recent years, there has been an increasing demand for miniaturization and high performance of a transformer, and in order to miniaturize the transformer, a grain-oriented electrical steel sheet is required to have exceptional high magnetic field iron loss such that iron loss is favorable even when magnetic flux density is high. At the same time, in recent years, it has been clarified that the forsterite film hinders movement of a magnetic domain wall and adversely affects iron loss. In a grain-oriented electrical steel sheet, a magnetic domain changes by movement of a magnetic domain wall under an alternating magnetic field. The smooth and rapid movement of the magnetic domain wall is effective for reducing iron loss, but the forsterite film itself is a non-magnetic body and has an uneven structure at the interface between the steel sheet and the coating, and it is considered that this uneven structure hinders the movement of the magnetic domain wall and thus adversely affects iron loss.

Therefore, as a means for improving high magnetic field iron loss, a technique for manufacturing a grain-oriented electrical steel sheet having no forsterite film (inorganic coating), or a technique for bringing a sheet surface into a mirror surface state (in other words, a technique for magnetically smoothing a sheet surface) have been studied by: removing a forsterite film by using a mechanical means such as polishing or a chemical means such as pickling; or preventing generation of a forsterite film in high-temperature finishing annealing.

As a technique for preventing the generation of a forsterite film, for example, Patent Document 2 discloses a technique in which a surface-formed product is removed through pickling after normal finishing annealing and then a sheet surface is brought into a mirror surface state through chemical polishing or electrolytic polishing. It has been found that a better iron loss improving effect can be obtained by forming a tension-applying insulating coating on the surface of a grain-oriented electrical steel sheet having no forsterite film, obtained by using such a known method. In addition, the tension-applying insulating coating can impart various characteristics such as corrosion resistance, heat resistance, and slippage in addition to improvement of iron loss.

However, the forsterite film has an effect of exhibiting an insulation property and an effect as an intermediate layer for securing adhesion when a tension coating (tension-applying insulating coating) is formed. That is, since the forsterite film is formed in a state of deeply entering the steel sheet, the forsterite film is exceptional in adhesion to the steel sheet which is metal. Therefore, when a tension applying type coating (tension coating) mainly containing colloidal silica, phosphate, or the like as a main component is formed on the surface of the forsterite film, the coating adhesion is exceptional. On the other hand, since it is generally difficult to bond a metal and an oxide, it is difficult to ensure sufficient adhesion between a tension coating and a sheet surface when a forsterite film is not present.

Thus, in the case of forming a tension coating on a grain-oriented electrical steel sheet having no forsterite film, it has been studied to provide a layer that substitutes for a role as an intermediate layer of a forsterite film.

For example, Patent Document 3 discloses a technique in which a grain-oriented electrical steel sheet having no forsterite film (inorganic film) is annealed in a weakly reducing atmosphere, and silicon inevitably contained in a silicon steel sheet is thermally oxidized selectively to form a SiO₂ layer on the sheet surface, and then a tension-applying type insulating coating is formed. In addition, Patent Document 4 discloses a technique in which a grain-oriented electrical steel sheet having no forsterite film (inorganic film) is subjected to an anodic electrolytic treatment in a silicate aqueous solution to form an SiO₂ layer on the sheet surface, and then a tension-applying type insulating coating is formed.

However, in the technique disclosed in Patent Document 3, it is necessary to prepare an annealing facility capable of controlling an atmosphere in order to perform annealing in a weakly reducing atmosphere, and there is a problem in treatment cost. In the technique disclosed in Patent Document 4, it is necessary to prepare a new electrolysis treatment facility in order to obtain a SiO₂ layer that maintains sufficient adhesion to a tension-applying type insulating coating on a sheet surface by performing an anodic electrolytic treatment in a silicate aqueous solution, and there is a problem in treatment cost.

On the other hand, Patent Document 5 discloses a grain-oriented electrical steel sheet including a base steel sheet and an insulating coating formed on a surface of the base steel sheet, in which the insulating coating is formed on the base steel sheet side and includes an intermediate layer containing a crystalline metal phosphate and a tension coating layer formed on a surface side of the insulating coating. In this grain-oriented electrical steel sheet, the intermediate layer can be formed through a chemical conversion treatment.

### Citation List

### Patent Documents

Patent Document 1: Japanese Unexamined Patent Application, First Publication No. S48-039338
Patent Document 2: Japanese Unexamined Patent Application, First Publication No. S49-96920
Patent Document 3: Japanese Unexamined Patent Application, First Publication No. H06-184762
Patent Document 4: Japanese Unexamined Patent Application, First Publication No. H11-209891
Patent Document 5: PCT International Publication No. WO 2022/215709

### SUMMARY OF INVENTION

### Technical Problem

In the technique in Patent Document 5, the intermediate layer made of a crystalline metal phosphate is provided between the base steel sheet and the tension coating, so that coating adhesion, coating tension, and magnetic characteristics can be improved. In addition, since the intermediate layer can be formed by chemical conversion treatment, no special facility is required. Therefore, this is a useful technique.

However, as a result of examination by the present inventors, it has been found that in the grain-oriented electrical steel sheet of Patent Document 5, when adhesion is improved, magnetic characteristics of a transformer may deteriorate. As a result of further studies on this point, it has been found that the cause of deterioration in magnetism is coarsening of crystals of the metal phosphate precipitated due to the chemical conversion treatment and a decrease in space factor when an actual transformer is produced.

Therefore, an object of the present invention is to provide a grain-oriented electrical steel sheet in which a layer containing a metal phosphate is formed on a surface of a steel sheet through chemical conversion treatment, the grain-oriented electrical steel sheet being exceptional in adhesion of a tension coating and magnetic characteristics and not reducing a space factor of a transformer (core). However, it is assumed that basic characteristics required for the coating, such as corrosion resistance and phosphoric acid dissolution resistance, do not deteriorate.

### Solution to Problem

The present inventors have found that when a layer containing a metal phosphate is provided as an intermediate layer for enhancing adhesion between a base steel sheet and a tension coating layer, coarsening of metal phosphate crystals can be curbed by containing a substance for curbing crystallization of phosphate in a chemical treatment liquid.

The present invention has been made in view of the above findings. The gist of the present invention is as follows.
[1] A grain-oriented electrical steel sheet according to an aspect of the present invention includes a base steel sheet; and an insulating coating formed on a surface of the base steel sheet, in which the insulating coating includes an intermediate layer formed on a side of the base steel sheet and containing a crystalline metal phosphate and one or more of amorphous silica, an inorganic filler, and a metal oxide, and a tension coating layer formed on a surface side of the insulating coating, and one or more of the amorphous silica, the inorganic filler, and the metal oxide has an average particle diameter of 10 to 500 nm.
[2] In the grain-oriented electrical steel sheet according to [1], the inorganic filler may contain one or two or more of alumina, BN, AlN, and kaolin.
[3] In the grain-oriented electrical steel sheet according to [1] or [2], the metal oxide may be one or two or more of titanium oxide, zinc oxide, and calcium oxide.
[4] In the grain-oriented electrical steel sheet according to any one of [1] to [3], the crystalline metal phosphate may have an average grain diameter of 1.0 to 12.0 µm.
[5] A method for forming an insulating coating according to another aspect of the present invention is a method for forming the insulating coating included in the grain-oriented electrical steel sheet according to [1], the method including a finishing annealing step of applying an annealing separator containing 10 to 100 mass% of Al₂O₃ to a steel sheet, drying the annealing separator, and then performing finishing annealing; an annealing separator removal step of removing an excess of the annealing separator from the steel sheet after the finishing annealing step; a light pickling step of pickling the steel sheet after the annealing separator removal step with a pickling liquid having a liquid temperature of 30 to 85°C and having 0.10 to 10.0 mass% of one inorganic acid selected from sulfuric acid, chloric acid, nitric acid, and phosphoric acid for 1 to 20 seconds; an immersion step of immersing the steel sheet after the light pickling step in a treatment liquid having a liquid temperature of 30 to 85°C and containing 0.3 to 10.0 mass% of a metal phosphate, 0.01 to 10.0 g/l of one or more of colloidal silica, an inorganic filler, and a metal oxide having an average particle diameter of 10 to 500 nm for 5 to 150 seconds; a drying step of pulling up the steel sheet after the immersion step from the treatment liquid, removing an excess of the treatment liquid, and then drying the steel sheet; and a tension coating layer forming step of applying, to the steel sheet after the drying step, a coating liquid containing a metal phosphate and colloidal silica such that a total concentration of the metal phosphate and the colloidal silica is 10 to 40 mass%, drying the coating liquid, then heating the steel sheet, and holding the steel sheet at a sheet temperature of 700 to 950°C for 10 to 50 seconds.

### Advantageous Effects of Invention

According to the above aspect of the present invention, it is possible to provide a grain-oriented electrical steel sheet which is exceptional in adhesion and magnetic characteristics of a tension coating and does not decrease a space factor of a transformer (core).

### BRIEF DESCRIPTION OF DRAWINGS

[FIG. 1] An example of a cross-sectional view of a grain-oriented electrical steel sheet according to the present embodiment.

### DESCRIPTION OF EMBODIMENTS

A grain-oriented electrical steel sheet according to an embodiment of the present invention (grain-oriented electrical steel sheet according to the present embodiment) and a method for manufacturing the grain-oriented electrical steel sheet according to the present embodiment, including a method for forming an insulating coating included in the grain-oriented electrical steel sheet according to the present embodiment, will be described.

First, the grain-oriented electrical steel sheet according to the present embodiment will be described.

As illustrated in FIG. 1, a grain-oriented electrical steel sheet 100 according to the present embodiment has a base steel sheet 1 and an insulating coating 2 formed on a surface of the base steel sheet 1. In the grain-oriented electrical steel sheet 100 according to the present embodiment, a forsterite film is not intentionally formed on the surface of the base steel sheet 1, and a forsterite film is not present in many cases. However, the presence of the forsterite film is acceptable as long as the coating mass is 1.0 g/m² or less (in that case, the forsterite film is present between the base steel sheet 1 and the insulating coating 2).

The insulating coating 2 has a tension coating layer 22 formed on a surface side of the insulating coating 2 (that is, a surface side of the grain-oriented electrical steel sheet 100), and an intermediate layer 21 formed on the base steel sheet 1 side and containing a crystalline metal phosphate.

In addition, the intermediate layer 21 contains a crystalline metal phosphate and one or more of amorphous silica, an inorganic filler, and a metal oxide, having an average particle diameter of 10 to 500 nm.

Each will be described below.

### <Base Steel Sheet>

### (Chemical Composition)

The grain-oriented electrical steel sheet 100 according to the present embodiment has a major feature in the structure of the insulating coating 2 formed on the surface of the base steel sheet 1, and the base steel sheet 1 included in the grain-oriented electrical steel sheet 100 is not limited in terms of its chemical composition. However, in order to obtain characteristics generally required for a grain-oriented electrical steel sheet, it is preferable to include the following components as chemical components. In the present embodiment, % relating to the chemical composition is mass% unless otherwise specified.

### C: 0.010% or less

C (carbon) is an element effective in controlling the microstructure of the steel sheet in steps up to completion of the decarburization annealing step in the manufacturing process. However, when the C content exceeds 0.010%, the magnetic characteristics of the grain-oriented electrical steel sheet, which is a product sheet, deteriorate. Therefore, in the base steel sheet of the grain-oriented electrical steel sheet according to the present embodiment, the C content is preferably 0.010% or less. The C content is more preferably 0.005% or less. The C content is preferably as low as possible, but even when the C content is reduced to less than 0.0001%, a microstructure control effect is saturated, and manufacturing cost is merely increased. Therefore, the C content may be 0.0001% or more.

### Si: 2.50 to 4.00%

Si (silicon) is an element that increases the electric resistance of a grain-oriented electrical steel sheet and improves iron loss characteristics. When the Si content is less than 2.50%, a sufficient eddy-current loss reducing effect cannot be obtained. Therefore, the Si content is preferably 2.50% or more. The Si content is more preferably 2.70% or more, and still more preferably 3.00% or more.

On the other hand, when the Si content exceeds 4.00%, the grain-oriented electrical steel sheet is embrittled, and passability significantly deteriorates. In addition, workability of the grain-oriented electrical steel sheet deteriorates, and the steel sheet may be fractured during rolling. Therefore, the Si content is preferably set to 4.00% or less. The Si content is more preferably 3.80% or less, and still more preferably 3.70% or less.

### Mn: 0.01 to 0.50%

Mn (manganese) is an element that is bonded to S in a manufacturing process to form MnS. This precipitate functions as an inhibitor (inhibitor of normal grain growth) and causes secondary recrystallization in steel. Mn is also an element that enhances hot workability of steel. When the Mn content is less than 0.01%, the above effect cannot be sufficiently obtained. Therefore, the Mn content is preferably 0.01% or more. The Mn content is more preferably 0.02% or more.

On the other hand, when the Mn content exceeds 0.50%, secondary recrystallization does not occur, and the magnetic characteristics of steel deteriorate. Therefore, in the base steel sheet of the grain-oriented electrical steel sheet according to the embodiment, the Mn content is preferably 0.50% or less. The Mn content is more preferably 0.20% or less, and still more preferably 0.10% or less.

### N: 0.010% or less

N (nitrogen) is an element that is bonded to Al in the manufacturing process to form AlN that functions as an inhibitor. However, when the N content exceeds 0.010%, the inhibitor excessively remains in the base steel sheet of the grain-oriented electrical steel sheet, and the magnetic characteristics deteriorate. Therefore, in the base steel sheet of the grain-oriented electrical steel sheet according to the embodiment, the N content is preferably 0.010% or less. The N content is more preferably 0.008% or less.

On the other hand, the lower limit value of the N content is not particularly limited, but even when the N content is reduced to less than 0.001%, manufacturing cost is merely increased. Therefore, the N content may be 0.001% or more.

### Sol. Al: 0.020% or less

Sol. Al (acid-soluble aluminum) is an element that is bonded to N in the manufacturing process of the grain-oriented electrical steel sheet to form AlN that functions as an inhibitor. However, when the sol. Al content in the base steel sheet exceeds 0.020%, the inhibitor excessively remains in the base steel sheet, so that magnetic characteristics deteriorate. Therefore, in the base steel sheet of the grain-oriented electrical steel sheet according to the embodiment, the sol. Al content is preferably 0.020% or less. The sol. Al content is more preferably 0.010% or less, and still more preferably less than 0.001%. The lower limit value of the sol. Al content is not particularly limited, but even when the content is reduced to less than 0.0001%, manufacturing cost is merely increased. Therefore, the sol. Al content may be 0.0001% or more.

### S: 0.010% or less

S (sulfur) is an element that is bonded to Mn in the manufacturing process to form MnS that functions as an inhibitor. However, when the S content exceeds 0.010%, the remaining inhibitor causes magnetic characteristics to deteriorate. Therefore, in the base steel sheet of the grain-oriented electrical steel sheet according to the present embodiment, the S content is preferably 0.010% or less. The S content in the grain-oriented electrical steel sheet is more preferably as low as possible. For example, the S content is less than 0.001%. However, even if the S content in the base steel sheet of the grain-oriented electrical steel sheet is reduced to less than 0.0001%, manufacturing cost is merely increased. Therefore, the S content in the base steel sheet of the grain-oriented electrical steel sheet may be 0.0001 % or more.

### Remainder: Fe and impurities

The chemical composition of the base steel sheet of the grain-oriented electrical steel sheet according to the present embodiment may contain the above-described elements, with the remainder of Fe and impurities. However, the base steel sheet may further contain Sn, Cu, Se, and Sb in the following ranges for the purpose of improving magnetic characteristics and the like. In addition, for example, even when the base steel sheet contains any one or more selected from W, Nb, Ti, Ni, Co, V, Cr, and Mo in a total amount of 1.0% or less as elements other than these elements, the effect of the grain-oriented electrical steel sheet according to the present embodiment is not impaired.

Here, the impurity is an element that is a contaminant derived from ore or scrap as a raw material, a manufacturing environment, or the like when the base steel sheet is industrially manufactured and means an element that is allowed to be included in a content that does not adversely affect the effect of the grain-oriented electrical steel sheet according to the embodiment.

### Sn: 0 to 0.50%

Sn (tin) is an element that contributes to improvement in magnetic characteristics through primary recrystallization structure control. In order to obtain an effect of improving magnetic characteristics, the Sn content is preferably 0.01% or more. The Sn content is more preferably 0.02% or more, and still more preferably 0.03% or more.

On the other hand, when the Sn content exceeds 0.50%, secondary recrystallization is unstable, and magnetic characteristics deteriorate. Therefore, the Sn content is preferably 0.50% or less. The Sn content is more preferably 0.30% or less, and still more preferably 0.10% or less.

### Cu: 0 to 0.50%

Cu (copper) is an element that contributes to an increase in Goss orientation occupancy in a secondary recrystallization structure. In order to obtain the above effect, the Cu content is preferably 0.01% or more. The Cu content is more preferably 0.02% or more, and still more preferably 0.03% or more.

On the other hand, when the Cu content exceeds 0.50%, the steel sheet is embrittled during hot rolling. Therefore, in the base steel sheet of the grain-oriented electrical steel sheet according to the embodiment, the Cu content is preferably 0.50% or less. The Cu content is more preferably 0.30% or less, and still more preferably 0.10% or less.

### Se: 0 to 0.020%

Se (selenium) is an element having an effect of improving magnetic characteristics. When Se is contained, the Se content is preferably 0.001% or more such that Se favorably exhibits the effect of improving magnetic characteristics. The Se content is more preferably 0.003% or more, and still more preferably 0.006% or more.

On the other hand, when the Se content exceeds 0.020%, adhesion of a coating deteriorates. Therefore, the Se content is preferably s 0.020% or less. The Se content is more preferably 0.015% or less, and still more preferably 0.010% or less.

### Sb: 0 to 0.50%

Sb (antimony) is an element having an effect of improving magnetic characteristics. When Sb is contained, the Sb content is preferably 0.005% or more such that Sb favorably exhibits the effect of improving magnetic characteristics. The Sb content is more preferably 0.01% or more, and still more preferably 0.02% or more.

On the other hand, when the Sb content exceeds 0.50%, adhesion of a coating significantly deteriorates. Therefore, the Sb content is preferably 0.50% or less. The Sb content is more preferably 0.30% or less, and still more preferably 0.10% or less.

As described above, for example, the chemical composition of the base steel sheet of the grain-oriented electrical steel sheet according to the present embodiment contains the above-described elements, with the remainder of Fe and impurities.

The chemical composition of the base steel sheet of the grain-oriented electrical steel sheet according to the present embodiment can be measured by using a known ICP emission spectrometry. Note that, at the time of measurement, in a case where an insulating coating is formed on a surface, the measurement is performed after the insulating coating is peeled off. As a peeling method, it is possible to peel off the insulating coating by immersing the base steel sheet with the insulating coating in a high-concentration alkaline solution (for example, a 30% sodium hydroxide solution heated to 85°C) for 20 minutes or more. It is possible to visually determine whether or not the insulating coating has been peeled off. In a case of a small sample, the insulating coating may be peeled off through surface grinding.

### <Insulating Coating>

In the grain-oriented electrical steel sheet 100 according to the present embodiment, the insulating coating 2 is formed on the surface of the base steel sheet 1.

The insulating coating 2 includes the intermediate layer 21 and the tension coating layer 22 in this order from the base steel sheet 1 side.

### (Intermediate Layer)

As described above, in general, a grain-oriented electrical steel sheet has a forsterite film generated in a finishing annealing step and an insulating coating (tension insulating coating) formed thereon. However, in recent years, it has been clarified that the forsterite film hinders movement of a magnetic domain wall and adversely affects iron loss, and thus, in order to further improve magnetic characteristics, a grain-oriented electrical steel sheet having no forsterite film has been studied. However, when the forsterite film is not present, it is difficult to ensure sufficient adhesion between a tension coating and a surface of a base steel sheet.

In the grain-oriented electrical steel sheet 100 according to the present embodiment, the intermediate layer 21 containing a crystalline metal phosphate is formed between the base steel sheet 1 and the tension coating to improve adhesion between the base steel sheet 1 and the tension coating layer 22 via the intermediate layer 21.

This is because when the intermediate layer 21 contains a crystalline metal phosphate, adhesion between the intermediate layer and the tension coating layer is exceptional because the tension coating (which becomes the tension coating layer 22 after formation) formed on the intermediate layer 21 also contains a metal phosphate and affinity is high. In addition, as will be described later, when the intermediate layer is formed by immersion in a treatment liquid containing a metal phosphate, the intermediate layer can be formed on a surface of the base steel sheet 1 using a chemical reaction, and adhesion between the intermediate layer 21 and the base steel sheet 1 can also be ensured.

When the intermediate layer 21 does not contain a crystalline metal phosphate, the above effect cannot be obtained. The proportion of the crystalline metal phosphate in the intermediate layer is preferably 80 mass% or more, preferably 90 mass% or more, and may be 99 mass% or more. The metal phosphate is preferably one or two or more of zinc phosphate, manganese phosphate, iron phosphate, and zinc calcium phosphate from the viewpoint of adhesion.

The intermediate layer may contain, as the remainder other than the metal phosphate, an oxide or an element diffused from the base steel sheet, such as Fe or Si.

However, when the crystal of the crystalline metal phosphate in the intermediate layer coarsens, the space factor decreases when an actual transformer is manufactured, so that the magnetic flux density per unit volume decreases and the transformer iron loss increases.

Therefore, in the grain-oriented electrical steel sheet according to the present embodiment, in order to curb the crystal coarsening by curbing the crystallization of the crystalline metal phosphate, one or more of colloidal silica, an inorganic filler, and a metal oxide having an average particle diameter of 10 to 500 nm are contained as an additive in the treatment liquid for forming an intermediate layer. As a result, an intermediate layer containing a crystalline metal phosphate and one or more of amorphous silica, an inorganic filler, and a metal oxide and in which an average particle diameter of one or more of amorphous silica, an inorganic filler, and a metal oxide is 10 to 500 nm, is formed as the intermediate layer. In such an intermediate layer, the average grain diameter of the crystalline metal phosphate is, for example, 1.0 to 12.0 µm.

It is preferable that one or more of the colloidal silica, the inorganic filler, and the metal oxide having an average particle diameter of 10 to 500 nm are not localized in the intermediate layer and are uniformly dispersed. For example, it is preferable that aggregates having a size of several µm or less are formed even when secondary aggregation occurs.

Among the amorphous silica, the inorganic filler, and the metal oxide added as an additive and remaining in the intermediate layer, the amorphous silica is preferable from the viewpoint of availability. The amorphous silica is different in form and effect from crystalline silica generated through thermal oxidation annealing or the like.

In addition, the inorganic filler preferably contains 90 mass% or more of one or two or more of alumina, BN, AlN, and kaolin (those having a purity of 90 mass% or more are used). BN preferably has a hexagonal crystal in consideration of ease of dispersion.

The metal oxide is preferably one or two or more of titanium oxide, zinc oxide, and calcium oxide from the viewpoint of stability of a treatment liquid.

A carbonate may be used as an additive, but the carbonate does not remain in the intermediate layer under normal baking conditions, and specific baking conditions are required to obtain an intermediate layer containing a carbonate, which is not preferable.

In addition, the content of one or more of the amorphous silica, the inorganic filler, and the metal oxide is preferably 0.01 to 1.00 mass%. When the content is less than 0.01 mass%, the effect of curbing crystal coarsening of the metal phosphate may be poor, and when the content is more than 1.00 mass%, the adhesion of an intermediate layer may be poor.

The intermediate layer 21 is formed at a timing different from that of the tension coating formed thereon, but both the intermediate layer 21 and the tension coating layer 22 exhibit an effect as the insulating coating 2.

The thickness of the intermediate layer is preferably 1.0 to 9.0 µm. When the average thickness of the intermediate layer 21 is less than 1.0 µm, the effect of improving the adhesion between the base steel sheet and the insulating coating via the intermediate layer may not be sufficiently obtained. On the other hand, when the average thickness of the intermediate layer is more than 9.0 µm, magnetic characteristics may deteriorate.

The mass proportion of the crystalline metal phosphate for the metal phosphate and the type of the metal phosphate in the intermediate layer can be obtained by measuring a cross section of the intermediate layer in the thickness direction by using a scanning electron microscope and an energy dispersive elemental analyzer. Whether the metal phosphate of the intermediate layer 21 is a crystalline metal phosphate can be determined according to X-ray crystallography.

The base steel sheet and the insulating coating can be discriminated on the basis of the concentration of P (phosphorus) (when the P content is 1.0 mass% or more, the insulating coating is determined, and when the P content is less than 1.0 mass%, the steel sheet is determined). In the insulating coating 2, the intermediate layer 21 and the tension coating layer 22 can be discriminated on the basis of the concentration difference of Si (when the Si content is 10 mass% or more, the tension coating layer is determined, and when the Si content is less than 10 mass%, the intermediate layer is determined).

The average grain diameter of the crystalline metal phosphate can be determined by using the following method.

The steel sheet is cut into a few mm square, which is easy to observe, and subjected to ion milling (CP processing) to remove micro shape defects such as shear droop and cracks, and then a cross section parallel to the rolling direction and the sheet thickness direction of the steel sheet and a cross section perpendicular to the rolling direction and parallel to the sheet thickness direction of the steel sheet are observed with a scanning electron microscope. The crystal form of the metal phosphate observed in the cross section is observed, and an average value of the major axis and minor axis of each crystal is measured for five or more of the cross sections, and the measured value is taken as a grain diameter. The electron microscope magnification at the time of observation is 1000 times.

In addition, the contents of the amorphous silica, the inorganic filler, and the metal oxide, and the average particle diameter can be determined according to the following method.

For the content, the steel sheet is cut into a few mm square, which is easy to observe, and subjected to ion milling (CP processing) to remove micro shape defects such as shear droop and cracks, and then a cross section parallel to the rolling direction and the sheet thickness direction of the steel sheet and a cross section perpendicular to the rolling direction and parallel to the sheet thickness direction of the steel sheet are observed with a scanning electron microscope at a magnification of 5000 times. The measurement is performed by analyzing a portion of the intermediate layer by using an energy dispersive elemental analyzer at five or more cross sections.

With regard to the average particle diameter, the presence of amorphous silica, an inorganic filler, and a metal oxide is confirmed at ten or more points in the intermediate layer through elemental analysis by using a transmission-type electron microscope for a cross-sectional sample subjected to ion milling in the same manner, and then an average value of the major axis and the minor axis of the particle observed at a magnification of 20,000 times is calculated as a particle diameter.

The thickness of the intermediate layer can be obtained according to the following method.

The total average thickness of the intermediate layer and the tension coating layer can be measured by observing the cross section of the sample with a scanning electron microscope and measuring the thickness at five or more points. The intermediate layer and the tension coating layer can be discriminated from each other on the basis of a concentration difference of silicon (Si) derived from silica. Therefore, the thickness of the intermediate layer can be calculated by subtracting the thickness of the tension coating layer from the total average thickness at each measurement point.

### (Tension Coating Layer)

The grain-oriented electrical steel sheet 100 according to the present embodiment has the tension coating layer 22 on a surface side of the insulating coating 2 by forming a tension coating on a surface of the intermediate layer 21.

The tension coating layer 22 is not particularly limited as long as it is used as an insulating coating of the grain-oriented electrical steel sheet, but from the viewpoint of adhesion to the intermediate layer 21 (adhesion to the base steel sheet 1 via the intermediate layer 21), it is preferable that the tension coating layer 22 has a composition containing a metal phosphate and silica as main components. It is more preferable to substantially contain a metal phosphate and silica.

The tension coating layer 22 preferably contains a metal phosphate and silica (derived from colloidal silica of the coating liquid) such that the content of silica is 20.0 mass% or more. On the other hand, when the silica content of the tension coating layer 22 is more than 60.0 mass%, it causes powdering, and thus it is preferable that the silica content is 60.0 mass% or less. In addition, it is preferable to contain the metal phosphate and silica are 70 mass% or more in total. The metal phosphate and silica may be 100 mass% in total. As the remainder other than the metal phosphate and silica, alumina or ceramic fine particles such as silicon nitride may be contained. The metal phosphate is preferably an aluminum phosphate from the viewpoint of heat resistance.

The thickness of the tension coating layer 22 is not limited, but the average thickness of the insulating coating 2 (the intermediate layer 21 + the tension coating layer 22) is preferably set to 1.0 to 20.0 µm when the average thickness of the intermediate layer 21 is in the above range. When the average thickness of the insulating coating 2 is less than 1.0 µm, a sufficient coating tension cannot be obtained. In addition, dissolution of phosphoric acid increases. In this case, this may cause stickiness and corrosion resistance deterioration and may cause coating peeling. On the other hand, when the thickness of the insulating coating 2 is more than 20.0 µm, a space factor decreases, so that magnetic characteristics deteriorate, or adhesion decreases due to cracks or the like, or corrosion resistance decreases.

In the tension coating layer 22, the mass ratio of the metal phosphate and the type of the metal phosphate can be determined in the same manner as in the intermediate layer in the cross section in the thickness direction.

As described above, the tension coating layer and the intermediate layer can be discriminated on the basis of the content of Si.

The thickness of the tension coating layer can be determined on the basis of in the same manner as in the intermediate layer. The sum of the thickness of the tension coating layer and the thickness of the intermediate layer is the thickness of the insulating coating.

### <Manufacturing Method>

According to a manufacturing method satisfying manufacturing conditions described below, the grain-oriented electrical steel sheet according to the present embodiment can be suitably manufactured. Note that, as a matter of course, the grain-oriented electrical steel sheet according to the present embodiment is not particularly limited in its manufacturing method. That is, a grain-oriented electrical steel sheet having the above-described configuration is regarded as the grain-oriented electrical steel sheet according to the present embodiment regardless of manufacturing conditions therefor.

The grain-oriented electrical steel sheet according to the present embodiment can be manufactured by using a manufacturing method including the following steps.
(I) a hot rolling step of hot-rolling a steel piece such as a slab having a predetermined chemical composition to obtain a hot rolled sheet;
(II) a hot-rolled sheet annealing step of annealing the hot rolled sheet;
(III) a cold rolling step of cold-rolling the hot rolled sheet after the hot-rolled sheet annealing step to obtain a steel sheet (cold rolled sheet);
(IV) a decarburization annealing step of performing decarburization annealing on the steel sheet after the cold rolling step;
(V) a finishing annealing step of applying an annealing separator containing 10 to 100 mass% of Al₂O₃ to the steel sheet, drying the annealing separator, and then performing finishing annealing;
(VI) an annealing separator removal step of removing an excess of the annealing separator from the steel sheet after the finishing annealing step;
(VII) a light pickling step of pickling the steel sheet after the annealing separator removal step with a pickling liquid having a liquid temperature of 30 to 85°C and having 0.10 to 10.0 mass% of one inorganic acid selected from sulfuric acid, chloric acid, nitric acid, and phosphoric acid for 1 to 20 seconds;
(VIII) an immersion step of immersing the steel sheet after the light pickling step in a treatment liquid having a liquid temperature of 30 to 85°C and containing 0.3 to 10.0 mass% of a metal phosphate, 0.01 to 10.0 g/l of one or more of colloidal silica, an inorganic filler, and a metal oxide having an average particle diameter of 10 to 500 nm for 5 to 150 seconds;
(IX) a drying step of pulling up the steel sheet after the immersion step from the treatment liquid, removing an excess of the treatment liquid, and then drying the steel sheet; and
(X) a tension coating layer forming step of applying, to the steel sheet after the drying step, a coating liquid containing a metal phosphate and colloidal silica such that a total concentration of the colloidal silica and the metal phosphate is 10 to 40 mass%, drying the coating liquid, then heating the steel sheet, and holding the steel sheet at a sheet temperature of 700 to 950°C for 10 to 50 seconds.

In addition, the method for manufacturing the grain-oriented electrical steel sheet according to the present embodiment may further include one or both of
(XI) a nitriding treatment step of subjecting the steel sheet to a nitriding treatment between the decarburization annealing step and the finishing annealing step, and
(XII) a magnetic domain refinement step of performing magnetic domain control of the steel sheet after the tension coating layer forming step.

Among them, the manufacturing method of the grain-oriented electrical steel sheet according to the present embodiment is characterized by the steps of (V) finishing annealing step to (X) tension coating layer forming step (collectively referred to as an insulating coating forming method) mainly related to formation of the insulating coating, and other steps or conditions not described can adopt known conditions.

Hereinafter, these steps will be described.

### [Hot Rolling Step]

In the hot rolling step, a steel piece having a predetermined chemical composition, such as a slab is heated and then hot-rolled to obtain a hot rolled sheet. The heating temperature of the steel piece is preferably in a range of 1100 to 1450°C. The heating temperature is more preferably 1300 to 1400°C.

The chemical composition of the steel piece may to be changed according to a chemical composition of a base steel sheet of a grain-oriented electrical steel sheet to be finally obtained, but examples thereof include a chemical composition containing, in mass%, C: 0.01 to 0.20%, Si: 2.50 to 4.00%, sol. Al: 0.01 to 0.040%, Mn: 0.01 to 0.50%, N: 0.020% or less, S: 0.005 to 0.040%, Cu: 0 to 0.50%, Sn: 0 to 0.50%, Se: 0 to 0.020%, and Sb: 0 to 0.50%, with the remainder of Fe and impurities.

The hot rolling conditions are not particularly limited, and is appropriately set according to required characteristics. The sheet thickness of the hot rolled sheet is preferably within a range of 2.0 to 3.0 mm, for example.

### [Hot-Rolled sheet Annealing Step]

The hot-rolled sheet annealing step is a step of annealing the hot rolled sheet manufactured through the hot rolling step. By performing such an annealing treatment, recrystallization occurs in the metallographic structure, and favorable magnetic characteristics can be preferably achieved.

When the hot-rolled sheet annealing is performed, the hot rolled sheet manufactured through the hot rolling step may be annealed according to a known method. The means for heating the hot rolled sheet at the time of annealing is not particularly limited, and a known heating method can be adopted. The annealing conditions are not particularly limited. For example, the hot rolled sheet can be annealed in a temperature range of 900 to 1200°C for 10 seconds to 5 minutes.

### [Cold Rolling Step]

**In** the cold rolling step, the hot rolled sheet after the hot-rolled sheet annealing step is subjected to cold rolling to obtain a steel sheet (cold rolled sheet). The cold rolling may be performed one time (continuously performed without intervening intermediate annealing(s)). Alternatively, before the final pass in the cold rolling step, intermediate annealing may be performed at least one time or two or more times by interrupting cold rolling, that is, cold rolling may be performed several times with intervening intermediate annealing(s).

When the intermediate annealing is performed, it is preferable to hold the hot rolled sheet at a temperature of 1000 to 1200°C for 5 to 180 seconds. The annealing atmosphere is not particularly limited. The number of times of intermediate annealing is preferably 3 or less in consideration of manufacturing cost.

In addition, before the cold rolling step, the surface of the hot rolled sheet may be subjected to pickling.

In the cold rolling step according to the present embodiment, the hot rolled sheet after the hot-rolled sheet annealing step is cold-rolled according to a known method to form a steel sheet. For example, the final rolling reduction can be in a range of 80 to 95%. When the final rolling reduction is 80% or more, a Goss nucleus in which the {110}<001> orientation has a high development degree in a rolling direction can be obtained, which is preferable. On the other hand, when the final rolling reduction exceeds 95%, there is a high possibility that secondary recrystallization is unstable in the subsequent finishing annealing step, which is not preferable.

The final rolling reduction is a cumulative rolling reduction of cold rolling, and when intermediate annealing is performed, the final rolling reduction is a cumulative rolling reduction of cold rolling after the final intermediate annealing.

### [Decarburization Annealing Step]

In the decarburization annealing step, the obtained steel sheet is subjected to decarburization annealing. In the decarburization annealing, decarburization annealing conditions are not limited as long as the steel sheet can be primarily recrystallized and C that adversely affects magnetic characteristics can be removed from the steel sheet, but for example, the steel sheet is held at an annealing temperature of 800 to 900°C for 10 to 600 seconds with a degree of oxidation (PH₂O/PH₂) of 0.3 to 0.6 in an annealing atmosphere (furnace atmosphere).

### [Nitriding Treatment Step]

A nitriding treatment may be performed between the decarburization annealing step and the finishing annealing step that will be described later.

In the nitriding treatment step, for example, the steel sheet after the decarburization annealing step is maintained at about 700 to 850°C in a nitriding treatment atmosphere (atmosphere containing a gas having nitriding ability, such as hydrogen, nitrogen, or ammonia) to perform the nitriding treatment. When AlN is utilized as an inhibitor, the N content of the steel sheet after the nitriding treatment step is preferably 40 ppm or more by the nitriding treatment. On the other hand, when the N content of the steel sheet after the nitriding treatment step exceeds 1000 ppm, AlN is excessively present in the steel sheet even after completion of secondary recrystallization in the finishing annealing. Such AlN causes iron loss deterioration. Therefore, the N content of the steel sheet after the nitriding treatment step is preferably 1000 ppm or less.

### [Finishing annealing Step]

In the finishing annealing step, an annealing separator containing 10 to 100 mass% of Al₂O₃ is applied to the steel sheet that is after the decarburization annealing step or has been further subjected to the nitriding treatment (after the nitriding treatment step), and dried, and then finishing annealing is performed.

In a conventional manufacturing method of a grain-oriented electrical steel sheet, a forsterite film is formed on the surface of a steel sheet (cold rolled sheet) by applying an annealing separator mainly containing MgO and performing finishing annealing. On the other hand, in the method for manufacturing the grain-oriented electrical steel sheet according to the present embodiment, an annealing separator containing Al₂O₃ is used so that a forsterite film is hardly formed.

On the other hand, the percentage of Al₂O₃ may be 100 mass% but, in the method for manufacturing the grain-oriented electrical steel sheet according to the present embodiment, the annealing separator preferably contains MgO from the viewpoint of preventing Al₂O₃ from burning into a sheet surface. MgO may be 0%, but the percentage of MgO is preferably set to 5 mass% or more when the above effect is to be obtained. When MgO is contained, the percentage of MgO is 90 mass% or less in order to secure 10 mass% or more of Al₂O₃. The percentage of MgO is preferably 50 mass% or less. Al₂O₃ and MgO may be more than 50 mass% in total in terms of solid content with respect to the annealing separator.

In addition, in the method for manufacturing the grain-oriented electrical steel sheet according to the present embodiment, the annealing separator may further contain a chloride. When the annealing separator contains a chloride, an effect that a forsterite film is more hardly formed can be obtained. The content of the chloride is not particularly limited, and may be 0%, but is preferably 0.5 to 10 mass% when the above effect is to be obtained. As the chloride, for example, bismuth chloride, calcium chloride, cobalt chloride, iron chloride, and nickel chloride are effective.

Finishing annealing conditions are not limited, but for example, a condition of holding the steel sheet at a temperature of 1150 to 1250°C for 10 to 60 hours can be adopted.

### [Annealing Separator Removal Step]

In the annealing separator removal step, an excess of the annealing separator is removed from the steel sheet after the finishing annealing step. For example, the excess of the annealing separator can be removed by performing water washing.

### [Light Pickling Step]

In the light pickling step, the steel sheet after the annealing separator removal step is subjected to pickling with 0.1 to 10.0 mass% of one inorganic acid selected from sulfuric acid, chloric acid, nitric acid, and phosphoric acid at a liquid temperature of 30 to 85°C for 1 to 20 seconds. The inorganic acid is preferably one selected from sulfuric acid, nitric acid, and phosphoric acid.

As a result, the effect of densifying the crystalline metal phosphate can be obtained.

When the light pickling conditions are not appropriate, the adhesion of the tension coating layer becomes poor or the dissolution resistance becomes poor.

### [Immersion Step]

### [Drying Step]

In the immersion step, the steel sheet after the light pickling step is immersed in the treatment liquid for 5 to 150 seconds, and in the drying step, the steel sheet after the immersion step is pulled up from the treatment liquid, the excess of the treatment liquid is removed, and then the steel sheet is dried. As a result, an intermediate layer is formed on the surface of the base steel sheet.

In the immersion step, the treatment liquid is adjusted to contain 0.3 to 10 mass% of a metal phosphate at a liquid temperature of 30 to 85°C, and 0.01 to 10.0 g/l of one or more of colloidal silica, an inorganic filler, and a metal oxide having an average particle diameter of 10 to 500 nm.

By containing one or more of colloidal silica (which becomes amorphous silica in the intermediate layer), an inorganic filler, and a metal oxide (which may be referred to as an additive), crystallization of the metal phosphate to be the intermediate layer is curbed, and as a result, the average grain diameter of the crystalline metal phosphate in the intermediate layer decreases.

However, when the content of the additive in the treatment liquid is less than 0.01 g/l, a sufficient effect cannot be obtained. On the other hand, when the content is more than 10.0 g/l, the treatment liquid becomes unstable.

When the average particle diameter of the additive is less than 10 nm, aggregation occurs and the treatment liquid becomes unstable. Alternatively, when the average particle diameter is more than 500 nm, the particles are precipitated and the dispersibility in the treatment liquid becomes poor.

When the liquid temperature of the treatment liquid is lower than 30°C or the treatment time is less than 5 seconds, the adhesion is poor. On the other hand, when the liquid temperature is higher than 85°C or the treatment time is longer than 150 seconds, the average grain diameter of the crystalline metal phosphate becomes too large.

On the other hand, when the content of the metal phosphate in the treatment liquid is more than 10 mass%, the average grain diameter of the metal phosphate may be coarsened to cause a decrease in adhesion. The metal phosphate contained in the treatment liquid may be one or two or more selected from zinc phosphate, manganese phosphate, and zinc calcium phosphate.

In addition, when the content of the metal phosphate in the treatment liquid is less than 0.3 mass%, formation of the intermediate layer is slow and cost is industrially high. When the film thickness of the intermediate layer is made uniform, the metal phosphate is preferably 1.0 mass% or more.

In addition, when the temperature at the time of drying is high, voids may be generated and adhesion may be poor, and thus the temperature at the time of drying is preferably 300°C or lower. The temperature is preferably 200°C or lower. The temperature at the time of drying is preferably 100°C or higher.

### [Tension Coating Layer Forming Step]

In the tension coating layer forming step, a coating liquid containing a metal phosphate and colloidal silica and having a total concentration of the metal phosphate and the colloidal silica of 10 to 40 mass% is applied to the steel sheet after the drying step, dried, and then heated and held for 10 to 50 seconds at a sheet temperature of 700 to 950°C to form a tension coating layer on the surface of the intermediate layer.

When the sheet temperature at the time of holding is lower than 700°C, the tension is low and the magnetic characteristics are poor. Therefore, the sheet temperature is preferably set to 700°C or higher. On the other hand, when the sheet temperature is higher than 950°C, rigidity of the steel sheet decreases and the steel sheet is easily deformed. In this case, the steel sheet may be distorted due to transfer or the like, resulting in poor magnetic characteristics. Therefore, the sheet temperature is preferably set to 950°C or lower.

When the holding time is less than 10 seconds, dissolution resistance is poor. Therefore, the holding time is set to 10 seconds or more. On the other hand, when the holding time is more than 50 seconds, adhesion of the tension coating layer is poor. Therefore, the holding time is preferably 50 seconds or less.

The coating liquid (insulating coating solution) contains 10 to 40 mass% of a metal phosphate and colloidal silica.

When the total concentration of the metal phosphate and the colloidal silica is less than 10 mass%, the applied treatment liquid easily flows, which causes an uneven application amount. On the other hand, when the content is more than 40 mass%, the viscosity becomes too high, which causes a pattern or coating unevenness.

As the metal phosphate, for example, one or a mixture of two or more selected from aluminum phosphate, zinc phosphate, magnesium phosphate, nickel phosphate, copper phosphate, lithium phosphate, and cobalt phosphate may be used. An aluminum phosphate is preferable from the viewpoint of stability of the treatment liquid.

The coating liquid may contain vanadium, tungsten, molybdenum, zirconium, and the like as additional elements. When these elements are contained, the elements may be added to the coating liquid, for example, as an oxygen acid.

As the colloidal silica, S-type or C-type colloidal silica may be used. The S-type colloidal silica means colloidal silica in which a silica solution is alkaline, and the C-type colloidal silica means colloidal silica in which a silica particle surface is subjected to an aluminum treatment, and a silica solution is alkaline to neutral. The S-type colloidal silica is widely and generally used, and is relatively inexpensive in price, but it is necessary to be careful because the S-type colloidal silica may aggregate and precipitate when being mixed with an acidic metal phosphate solution. The C-type colloidal silica is stable even when being mixed with a metal phosphate solution, and there is no possibility of precipitation, but the C-type colloidal silica is relatively expensive because the number of treatment steps is large. It is preferable to select and use them according to the stability of a coating liquid to be prepared.

### [Magnetic Domain Refinement Step]

The method for manufacturing the grain-oriented electrical steel sheet according to the present embodiment may further include a magnetic domain refinement step of performing magnetic domain refinement on the steel sheet after the tension coating layer forming step.

By performing the magnetic domain refinement treatment, iron loss of the grain-oriented electrical steel sheet can be further reduced.

The method of the magnetic domain refinement treatment include: a method for narrowing the width of a 180° magnetic domain (performing refinement of a 180° magnetic domain) by forming linear or dotted groove parts extending in a direction intersecting a rolling direction at predetermined intervals in the rolling direction; and a method for narrowing the width of a 180° magnetic domain (performing refinement of a 180° magnetic domain) by forming linear or dotted stress-strain parts or groove parts extending in a direction intersecting a rolling direction at predetermined intervals in the rolling direction.

In a case where a stress-strain part is formed, laser beam irradiation, electron beam irradiation, and the like can be applied. In a case where a groove part is formed, a mechanical groove forming method using a blade-like or the like, a chemical groove forming method by electrolytic etching, a thermal groove forming method by laser irradiation, and the like can be applied.

In a case where the insulating coating is damaged due to formation of a stress-strain part or a groove part and characteristics such as insulation properties are deteriorated, the insulating coating may be formed again to repair the damage.

### Examples

A slab containing, in mass%, C: 0.08%, Si: 3.31%, sol. Al: 0.028% N: 0.008%, Mn: 0.07%, and S: less than 0.0005%, with the remainder of Fe and impurities, was cast.

The slab was heated to 1350°C and then hot-rolled to obtain a hot rolled sheet having a sheet thickness of 2.2 mm.

The hot rolled sheet was annealed under the condition of being held at 1100°C for 10 seconds. (Hot Rolled sheet Annealing)

Thereafter, the hot rolled sheet was cold-rolled to obtain a cold rolled sheet having a sheet thickness of 0.22 mm.

The cold rolled sheet was subjected to decarburization annealing under the condition of being held at 830°C for 90 seconds.

After the decarburization annealing, an annealing separator containing 45 mass% of MgO, 50 mass% of Al₂O₃, and 5 mass% of BiCl₃ as a bismuth chloride was applied and dried, and then finishing annealing was performed at 1200°C for 20 hours.

After the finishing annealing, the steel sheet was washed with water to remove an excess of the annealing separator, and as a result, a forsterite film was not formed on the sheet surface.

The steel sheet was subjected to light pickling under the conditions in Table 2-1.

After light pickling, an intermediate layer was formed by using a treatment liquid in which a phosphate and an additive shown in Table 1 were mixed. The drying temperature was 200°C. The obtained intermediate layer was as shown in Table 2-2. The proportion of the crystalline metal phosphate in the intermediate layer was 80 mass% or more.

Thereafter, an insulating coating treatment liquid containing a metal phosphate and colloidal silica shown in Table 2-3 as main components was applied, and dried at 850°C for 20 seconds after the application to form a tension coating layer on the sheet surface.

The thickness of the insulating coating (the intermediate layer and the tension coating layer) were as shown in Table 2-3. The tension coating layer was substantially composed of a metal phosphate and silica.

**[Table 1]**

| Intermediate Layer NO. | Immersion Step | | | | | | |
|---|---|---|---|---|---|---|---|
| | Treatment Liquid | | | | | Treatment Conditions | |
| | Metal Phosphate | | Additive | | | Treatment Liquid Temperature (°C) | Immersion Time (sec) |
| | Type | Content (mass%) | Type | Average Particle diameter (nm) | Compounded Amount (g/l) | | |
| 1 | Zinc Phosphate | 3.5 | Colloidal Silica | 20 | 0.5 | 40 | 20 |
| 2 | Zinc Phosphate | 2.5 | Colloidal Silica | 30 | 1.0 | 30 | 20 |
| 3 | Manganese Phosphate | 10.0 | Colloidal Silica | 45 | 2.0 | 85 | 10 |
| 4 | Manganese Phosphate | 7.5 | Colloidal Titanium Oxide | 40 | 0.5 | 80 | 20 |
| 5 | Zinc Calcium Phosphate | 5.5 | Zinc Oxide Colloid Particle | 40 | 1.5 | 80 | 12 |
| 6 | Zinc Phosphate | 1.0 | Zirconia Sol | 200 | 5.0 | 40 | 5 |
| 7 | Manganese Phosphate | 4.0 | Alumina Sol | 40 | 1.5 | 60 | 5 |
| 8 | Zinc Phosphate | 1.5 | Aluminum Nitride Particle | 50 | 1.0 | 50 | 120 |
| 9 | Manganese Phosphate | 8.5 | BN Slurry | 50 | 1.0 | 85 | 40 |
| 10 | Zinc Phosphate | 1.8 | Kaolin Particle | 100 | 6.5 | 40 | 100 |
| 11 | Zinc Phosphate | 2.0 | Alumina Particle | 500 | 12.0 | 40 | 10 |
| 12 | Manganese Phosphate | 6.5 | Particulate Silica | 2100 | 5.5 | 60 | 40 |
| 13 | Zinc Phosphate | 1.5 | Colloidal Silica | 8 | 0.05 | 50 | 10 |
| 14 | Zinc Phosphate | 1.5 | Colloidal Silica | 20 | 0.50 | 50 | 4 |
| 15 | Manganese Phosphate | 4.0 | - | - | - | 55 | 150 |

**[Table 2-1]**

| No. | Light Pickling Step | | | | Intermediate Layer Forming Conditions |
|---|---|---|---|---|---|
| | Type of Acid | Concentration (mass%) | Temperature (°C) | Time (sec) | Intermediate Layer No. |
| 1 | H₂SO₄ | 2.5 | 85 | 5 | 1 |
| 2 | H₂SO₄ | 1.0 | 85 | 10 | 2 |
| 3 | H₃PO₄ | 1.5 | 65 | 5 | 3 |
| 4 | H₂SO₄ | 0.5 | 80 | 20 | 4 |
| 5 | H₂SO₄ | 3.5 | 80 | 5 | 5 |
| 6 | H₃PO₄ | 3.0 | 50 | 10 | 6 |
| 7 | H₃PO₄ | 2.5 | 60 | 15 | 7 |
| 8 | H₃PO₄ | 0.8 | 55 | 20 | 8 |
| 9 | HNO₃ | 0.5 | 40 | 10 | 9 |
| 10 | HNO₃ | 0.5 | 35 | 10 | 10 |
| 11 | H₃PO₄ | 1.0 | 80 | 10 | 11 |
| 12 | H₂SO₄ | 0.5 | 60 | 10 | 12 |
| 13 | H₃PO₄ | 1.0 | 80 | 10 | 13 |
| 14 | H₂SO₄ | 0.5 | 60 | 10 | 14 |
| 15 | H₂SO₄ | 0.5 | 60 | 10 | 15 |
| 16 | H₂SO₄ | 0.02 | 80 | 10 | 1 |
| 17 | H₂SO₄ | 1.5 | 25 | 10 | 1 |
| 18 | H₂SO₄ | 0.5 | 94 | 10 | 1 |
| 19 | H₃PO₄ | 2.5 | 55 | 0.4 | 3 |
| 20 | H₃PO₄ | 2.5 | 55 | 60 | 3 |
| 21 | HCl | 0.5 | 35 | 20 | 3 |

**[Table 2-2]**

| No. | Intermediate Layer | | | | | |
|---|---|---|---|---|---|---|
| | Crystalline Metal Phosphate | | Thickness | Amorphous Silica, Inorganic Filler, and/or Metal Oxide | | |
| | Type | Average Grain diameter (µm) | (µm) | Type | Average Particle diameter (nm) | Content (mass%) |
| 1 | Zinc Phosphate | 4.5 | 6.2 | Amorphous Silica | 20 | 0.20 |
| 2 | Zinc Phosphate | 6.8 | 6.8 | Amorphous Silica | 30 | 0.30 |
| 3 | Manganese Phosphate | 8.9 | 7.4 | Amorphous Silica | 45 | 0.70 |
| 4 | Manganese Phosphate | 9.4 | 8.4 | Titanium Oxide | 40 | 0.40 |
| 5 | Zinc Phosphate, Calcium Phosphate | 8.4 | 8.7 | Zinc Oxide | 40 | 0.05 |
| 6 | Zinc Phosphate | 3.1 | 3.6 | Zirconia | 200 | 0.02 |
| 7 | Manganese Phosphate | 8.8 | 8.8 | Alumina | 40 | 0.40 |
| 8 | Zinc Phosphate | 2.6 | 3.3 | AlN | 50 | 0.02 |
| 9 | Manganese Phosphate | 9.7 | 8.9 | Boron Nitride | 50 | 0.10 |
| 10 | Zinc Phosphate | 6.7 | 8.3 | Kaolin | 100 | 0.50 |
| 11 | Zinc Phosphate | 0.9 | 2.2 | - | - | - |
| 12 | Zinc Phosphate | 14.3 | 21.3 | Silica(Crystalline) | 2100 | 0.20 |
| 13 | Zinc Phosphate | 0.6 | 0.9 | Amorphous Silica | 8 | 0.01 |
| 14 | Zinc Phosphate | 0.4 | 0.9 | - | - | - |
| 15 | Manganese Phosphate | 16.3 | 19.2 | - | - | - |
| 16 | Zinc Phosphate | 12.7 | 6.3 | Amorphous Silica | 10 | 0.001 |
| 17 | Zinc Phosphate | 13.4 | 6.6 | - | - | - |
| 18 | Zinc Phosphate | 12.4 | 5.8 | Amorphous Silica | 20 | 0.003 |
| 19 | Manganese Phosphate | 15.6 | 6.9 | - | - | - |
| 20 | Manganese Phosphate | 15.6 | 7.1 | Amorphous Silica | 40 | 0.001 |
| 21 | Manganese Phosphate | 14.9 | 7.4 | - | - | - |

**[Table 2-3]**

| No. | Tension Coating Layer Forming Step | | | | | Tension Coating Layer | Insulating Coating | Remarks |
|---|---|---|---|---|---|---|---|---|
| | Coating Liquid | | | | | Silica Content (mass%) | Thickness (µm) | |
| | Metal Phosphate(100 parts by mass) | Metal Element Molar Ratio | Colloidal Silica | | Total Concentration of Metal Phosphate and Colloidal Silica (mass%) | | | |
| | Type | | Type | parts by mass | | | | |
| 1 | Aluminum Phosphate | - | S Type | 90 | 35 | 47.4 | 9.5 | Invention Example |
| 2 | Zinc Phosphate | - | S Type | 60 | 36 | 37.5 | 10.1 | Invention Example |
| 3 | Aluminum/Zinc Phosphate | 0.25 | C Type | 140 | 25 | 58.3 | 10.7 | Invention Example |
| 4 | Aluminum/Copper Phosphate | 0.17 | S Type | 100 | 34 | 50.0 | 11.7 | Invention Example |
| 5 | Aluminum/Lithium Phosphate | 0.15 | S Type | 80 | 35 | 44.4 | 12.0 | Invention Example |
| 6 | Aluminum/Barium Phosphate | 0.15 | C Type | 75 | 28 | 42.9 | 6.9 | Invention Example |
| 7 | Aluminum/Molybdenum Phosphate | 0.14 | C Type | 100 | 27 | 50.0 | 12.1 | Invention Example |
| 8 | Aluminum/Vanadium Phosphate | 0.14 | C Type | 80 | 28 | 44.4 | 6.6 | Invention Example |
| 9 | Aluminum/Tungsten Phosphate | 0.17 | C Type | 130 | 26 | 56.5 | 12.2 | Invention Example |
| 10 | Aluminum/Zirconium Phosphate | 0.17 | C Type | 60 | 29 | 37.5 | 11.6 | Invention Example |
| 11 | Aluminum/Copper Phosphate | 0.17 | S Type | 60 | 36 | 37.5 | 4.7 | Comparative Example |
| 12 | Aluminum/Copper Phosphate | 0.17 | S Type | 90 | 35 | 47.4 | 24.6 | Comparative Example |
| 13 | Aluminum/Copper Phosphate | 0.17 | S Type | 60 | 36 | 37.5 | 20.1 | Comparative Example |
| 14 | Aluminum/Copper Phosphate | 0.17 | C Type | 100 | 27 | 50.0 | 4.2 | Comparative Example |
| 15 | Aluminum/Copper Phosphate | 0.17 | C Type | 100 | 27 | 50.0 | 22.5 | Comparative Example |
| 16 | Aluminum/Vanadium Phosphate | 0.14 | C Type | 80 | 28 | 44.4 | 9.6 | Comparative Example |
| 17 | Aluminum/Vanadium Phosphate | 0.14 | C Type | 80 | 28 | 44.4 | 9.7 | Comparative Example |
| 18 | Aluminum/Vanadium Phosphate | 0.14 | C Type | 80 | 28 | 44.4 | 9.1 | Comparative Example |
| 19 | Aluminum/Barium Phosphate | 0.15 | C Type | 75 | 28 | 42.9 | 7.5 | Comparative Example |
| 20 | Aluminum/Barium Phosphate | 0.15 | C Type | 75 | 28 | 42.9 | 13.2 | Comparative Example |
| 21 | Aluminum/Copper Phosphate | 0.17 | S Type | 100 | 34 | 50.0 | 8.2 | Comparative Example |

The obtained steel sheet (grain-oriented electrical steel sheet) was irradiated with a laser beam under the conditions that UA (irradiation energy density) was 2.0 J and an irradiation interval was 5.0 mm pitch to perform a magnetic domain refinement treatment.

The iron loss W17/50 (iron loss at 50 Hz at 1.7 T) of the steel sheet after the magnetic domain refinement treatment was measured by using a single sheet tester (SST) according to JIS C2556 (2015).

In addition, the space factor was measured in the following manner.

### [Space Factor]

The space factor was measured by using a method in accordance with JIS C 2550-5 (2020). 30 test pieces having a width of 30 mm and a length of 320 mm were used. The total mass of the sample was measured, and then the total mass of the sample was calculated by measuring between the upper and lower contact sheets sandwiching the laminated body in a state of being pressurized at 1 MPa.

When the space factor was 96.0% or more, it was determined that a high space factor was secured.

In addition, coating adhesion, coating tension, corrosion resistance, and dissolution resistance of the steel sheet after the magnetic domain refinement treatment were evaluated according to the following methods. Table 3 shows the results.

### [Coating Adhesion]

Adhesion of a coating was evaluated by the degree of peeling (area ratio) of the coating after a bending adhesion test was performed in which a sample having a width of 30 mm and a length of 300 mm was collected from a steel sheet, the sample was subjected to stress relief annealing at 800°C for two hours in a nitrogen stream, and then wound around a 10 mmφ cylinder and unwound.

The evaluation criteria were as follows, and in the case of A or B, it was determined that the coating adhesion was exceptional.
A: Peeling area ratio of 0 to 0.5%
B: Peeling area ratio of more than 0.5% and 5.0% or less
C: Peeling area ratio of more than 5.0% and 20% or less
D: Peeling area ratio of more than 20% and 50% or less
E: Peeling area ratio of more than 50%

### [Coating Tension]

The coating tension was calculated by back calculation from the curved state when one surface of the insulating coating was peeled off. When the obtained coating tension was 4.0 MPa or more, it was determined that the coating had a sufficient coating tension.

### [Corrosion Resistance]

Regarding corrosion resistance, a 5%NaCl aqueous solution was naturally dropped to a sample for 7 hours in an atmosphere at 35°C according to a salt spray test (JIS Z2371:2015) of JIS method.

Thereafter, a rusting area was evaluated at 10 points. The evaluation criteria were as follows. A score of 5 or more (5 to 10) was determined to be exceptional in corrosion resistance.
10: No rust was generated
9: Rust was generated in an extremely small amount (area ratio was 0.10% or less)
8: Rust was generated in an area ratio of more than 0.10% and 0.25% or less
7: Rust was generated in an area ratio of more than 0.25% and 0.50% or less
6: Rust was generated in an area ratio of more than 0.50% and 1.0% or less
5: Rust was generated in an area ratio of more than 1.0% and 2.5% or less
4: Rust was generated in an area ratio of more than 2.5% and 5.0% or less
3: Rust was generated in an area ratio of more than 5.0% and 10% or less
2: Rust was generated in an area ratio of more than 10% and 25% or less
1: Rust was generated in an area ratio of more than 25% and 50% or less

### [Dissolution Resistance]

The dissolution resistance was evaluated by whether or not the dissolution of phosphoric acid from the sample could be curbed.

The dissolution amount was measured by boiling the sample in boiled pure water for 10 minutes, measuring the amount of phosphoric acid eluted in the pure water, and dividing the amount of phosphoric acid by the area of the insulating coating of the boiled grain-oriented electrical steel sheet. The amount of phosphoric acid eluted in the pure water was calculated by cooling the pure water (solution) in which phosphoric acid was eluted, diluting the cooled solution with pure water, and measuring the phosphoric acid concentration of the sample by using ICP-AES.

When the dissolution amount was less than 40 mg/m², it was determined that the dissolution resistance was exceptional.

**[Table 3]**

| No. | Coating Adhesion | Coating Tension MPa | Corrosion Resistance | Dissolution Resistance mg/m² | Space Factor (%) | Iron Loss(W17/50) W/Kg | Remarks |
|---|---|---|---|---|---|---|---|
| 1 | B | 7.6 | 8 | 24 | 96.4 | 0.66 | Invention Example |
| 2 | B | 7.4 | 8 | 31 | 96.6 | 0.64 | Invention Example |
| 3 | A | 8.9 | 7 | 21 | 96.8 | 0.59 | Invention Example |
| 4 | A | 8.9 | 7 | 20 | 96.2 | 0.62 | Invention Example |
| 5 | A | 9.2 | 9 | 31 | 97.2 | 0.64 | Invention Example |
| 6 | B | 6.8 | 9 | 28 | 97.4 | 0.68 | Invention Example |
| 7 | B | 9.8 | 7 | 27 | 96.1 | 0.59 | Invention Example |
| 8 | B | 6.9 | 8 | 22 | 97.7 | 0.64 | Invention Example |
| 9 | A | 9.4 | 7 | 19 | 96.0 | 0.61 | Invention Example |
| 10 | B | 6.1 | 9 | 23 | 96.5 | 0.69 | Invention Example |
| 11 | C | 3.9 | 8 | 27 | 96.8 | 0.73 | Comparative Example |
| 12 | B | 7.7 | 7 | 56 | 91.2 | 0.71 | Comparative Example |
| 13 | B | 4.3 | 8 | 45 | 91.8 | 0.77 | Comparative Example |
| 14 | A | 8.4 | 5 | 48 | 97.1 | 0.71 | Comparative Example |
| 15 | B | 7.8 | 5 | 44 | 92.2 | 0.72 | Comparative Example |
| 16 | C | 5.3 | 4 | 25 | 96.1 | 0.78 | Comparative Example |
| 17 | C | 4.9 | 4 | 32 | 95.6 | 0.73 | Comparative Example |
| 18 | B | 6.7 | 7 | 42 | 95.8 | 0.69 | Comparative Example |
| 19 | D | 2.7 | 5 | 39 | 96.6 | 0.72 | Comparative Example |
| 20 | B | 7.1 | 4 | 51 | 94.3 | 0.75 | Comparative Example |
| 21 | D | 3.3 | 4 | 35 | 96.0 | 0.74 | Comparative Example |

As can be seen from Tables 1 to 3, in the present invention examples, the coating main characteristics including adhesion are extremely exceptional, and the iron loss and the space factor are improved.

On the other hand, in the comparative examples, the insulating coating did not have a preferable composition, and the tension coating was poor in one or more of adhesion, magnetic characteristics, corrosion resistance, phosphoric acid dissolution resistance, and a space factor of a transformer (core).

### INDUSTRIAL APPLICABILITY

According to the present invention, it is possible to provide a grain-oriented electrical steel sheet which is exceptional in adhesion and magnetic characteristics of a tension coating and does not decrease a space factor of a transformer (core). Therefore, industrial applicability is high.

### REFERENCE SIGNS LIST

100 Grain-oriented electrical steel sheet
1 Base steel sheet
2 Insulating coating
21 Intermediate layer
22 Tension coating layer

## Claims

1. A grain-oriented electrical steel sheet comprising:
a base steel sheet; and
an insulating coating formed on a surface of the base steel sheet, wherein
the insulating coating includes:
an intermediate layer formed on a side of the base steel sheet and containing a crystalline metal phosphate and one or more of amorphous silica, an inorganic filler, and a metal oxide, and
a tension coating layer formed on a surface side of the insulating coating, and
one or more of the amorphous silica, the inorganic filler, and the metal oxide has an average particle diameter of 10 to 500 nm.

2. The grain-oriented electrical steel sheet according to claim 1, wherein the inorganic filler contains one or two or more of alumina, BN, AlN, and kaolin.

3. The grain-oriented electrical steel sheet according to claim 1 or 2, wherein
the metal oxide is one or two or more of titanium oxide, zinc oxide, and calcium oxide.

4. The grain-oriented electrical steel sheet according to claim 1 or 2, wherein
the crystalline metal phosphate has an average grain diameter of 1.0 to 12.0 µm.

5. A method for forming the insulating coating included in the grain-oriented electrical steel sheet according to claim 1, the method comprising:
a finishing annealing step of applying an annealing separator containing 10 to 100 mass% of Al₂O₃ to a steel sheet, drying the annealing separator, and then performing finishing annealing;
an annealing separator removal step of removing an excess of the annealing separator from the steel sheet after the finishing annealing step;
a light pickling step of pickling the steel sheet after the annealing separator removal step with a pickling liquid having a liquid temperature of 30 to 85°C and having 0.10 to 10.0 mass% of one inorganic acid selected from sulfuric acid, chloric acid, nitric acid, and phosphoric acid for 1 to 20 seconds;
an immersion step of immersing the steel sheet after the light pickling step in a treatment liquid having a liquid temperature of 30 to 85°C and containing 0.3 to 10.0 mass% of a metal phosphate, 0.01 to 10.0 g/l of one or more of colloidal silica, an inorganic filler, and a metal oxide having an average particle diameter of 10 to 500 nm for 5 to 150 seconds;
a drying step of pulling up the steel sheet after the immersion step from the treatment liquid, removing an excess of the treatment liquid, and then drying the steel sheet; and
a tension coating layer forming step of applying, to the steel sheet after the drying step, a coating liquid containing a metal phosphate and colloidal silica such that a total concentration of the metal phosphate and the colloidal silica is 10 to 40 mass%, drying the coating liquid, then heating the steel sheet, and holding the steel sheet at a sheet temperature of 700 to 950°C for 10 to 50 seconds.
